

1

3,001,938

LUBRICANTS CONTAINING SALTS OF ORGANIC-SUBSTITUTED PHOSPHORUS - CONTAINING ACIDS

Arnold J. Morway, Clark, and Jeffrey H. Bartlett, New Providence, N.J., assignors to Esso Research and Engineering Company, a corporation of Delaware  
No Drawing. Filed Apr. 1, 1958, Ser. No. 725,489  
12 Claims. (Cl. 252—32.5)

This invention relates to lubricating compositions containing salts of phosphonic and phosphinic acids. Particularly, it relates to greases and lubricating fluids containing complexes of salts of carboxylic acids and salts of a hydroxy alkyl phosphonic acid and/or a salt of a hydroxy alkyl phosphinic acid, wherein said phosphorus-containing acid has a carbon atom content of 1 to 5.

This application is a continuation-in-part of our prior pending application Serial Number 654,981, filed April 25, 1957, and now abandoned.

Mixed salt complexes comprising salts of low molecular weight carboxylic acid in combination with salts of intermediate and/or high molecular weight carboxylic acid, are known. These prior complexes have been used as grease thickeners and for imparting certain desirable properties to fluid-type lubricants. However, it has now been found that greases and lubricating fluids may be prepared from complexes of salts of hydroxy alkyl phosphonic or phosphinic acid in various combinations with salts of low molecular weight carboxylic acid, intermediate and high molecular weight carboxylic acid. This new type of complex may be incorporated in lubricating oil in amounts of about 20 to 30 weight percent, based on the total composition, to form greases having higher load-carrying ability, reduced wear characteristics and a higher degree of thixotropy than greases thickened with the aforementioned prior complexes. By using smaller amounts, such as 5 to 10 weight percent of the complex of the invention, fluid lubricants may be formed which also have high load-carrying ability and reduced wear properties. Furthermore, the presence of the phosphonic or phosphinic acid salt in the complex acts as a color stabilizer and oxidation inhibitor. In addition, the salts of the phosphorus-containing acids tend to prevent crust formation and/or undue hardening of the greases during storage, particularly when soaps of high molecular weight fatty acids ( $C_{18+}$ ) are present in the complex.

The hydroxy alkyl phosphonic or phosphinic acids utilized in the present invention can be defined by the general formula:



wherein R is hydrogen or a  $C_1$  to  $C_4$  alkyl group and R' may be either hydrogen or an alkyl radical containing from 1 to 5, preferably 0 to 3, carbon atoms. The total number of carbon atoms in the compound should be about 1 to 5. X may be a hydroxyl group, in which case the formula represents a phosphonic acid, or X may be hydrogen whereupon the formula represents a phosphinic acid. These compounds and their method of preparation

2

are known to the art. Examples of specific compounds which may be used include:

- 1-hydroxy-1-methylethylphosphonic acid
- 1-hydroxyethylphosphonic acid
- 5 1-hydroxy-1-methylpropylphosphonic acid
- 1-hydroxy-2-methylpropylphosphonic acid
- 1-hydroxybutylphosphinic acid
- 1-hydroxymethylphosphinic acid
- 1-hydroxy-1-ethylpropylphosphonic acid
- 10 1-hydroxy-3-methylbutylphosphinic acid
- 1-hydroxypropylphosphonic acid

Low molecular weight acids suitable for the complex formation include saturated and unsaturated, substituted and unsubstituted aliphatic monocarboxylic acids having about 1 to 6 carbon atoms. These acids include fatty acids such as formic, acetic, propionic, furoic, acrylic, and similar acids including their hydroxy derivatives such as lactic acid, etc. Acetic acid or its anhydride is preferred. Mixtures of these low molecular weight acids may be employed if desired.

Intermediate molecular weight fatty acids which may be used include those aliphatic, saturated or unsaturated, unsubstituted, monocarboxylic acids containing 7 to 12 carbon atoms per molecule, e.g. capric, caprylic, nonanoic acid, lauric acid, etc.

The high molecular weight fatty acids or aliphatic monocarboxylic acids useful for forming the complexes of the invention include naturally-occurring or synthetic, substituted and unsubstituted, saturated and unsaturated, fatty acids having about 16 to 30, e.g. 16 to 22, carbon atoms per molecule. Examples of such acids include palmitic, stearic, dihydroxy stearic, behenic, montanic, linolinic, linoleic, arachidic, ricinoleic, oleic, hydrogenated fish oil, tallow acids, etc.

The metal component of the complex thickeners of this invention may be either an alkali metal such as lithium, potassium, sodium or an alkaline earth metal such as calcium, strontium, barium and magnesium. Mixtures of the grease-forming metals may be employed if desired. The metals are usually reacted with the acids in the form of metal bases, such as hydroxides, oxides, carbonates, etc.

The compositions of the invention will comprise a major proportion of a lubricating oil and about 5 to 30 weight percent of the complex material. When a grease is desired, the composition will contain about 10 to 30, e.g. 15 to 25, weight percent of the complex, while in the case of fluid lubricants, the composition will contain about 5 to 15, e.g. 5 to 10, weight percent of the complex. All of said weight percentages are based on the total weight of the composition.

The thickener, in turn, will contain the salts of about .1 to 10, e.g. .3 to 5.0, moles of the high and/or intermediate molecular weight fatty acid per one mole of phosphonic or phosphinic acid. If the salt of a low molecular weight carboxylic acid is also used in the preparation of the complex, then it will be present in ratios of about 5:1 to 30:1, e.g. 5:1 to 20:1, moles of the low molecular weight carboxylic acid per one mole of the phosphonic or phosphinic acid. In terms of parts by weight, excellent mixed-salt complexes may be prepared from a mixture of 0.2 to 5.0, e.g. 0.5 to 4.0, parts of the phosphonic or phosphinic acid, 1 to 20 parts by weight of either high or intermediate molecular weight fatty acid or mixtures in any proportion of said high and intermediate molecular weight fatty acids.

mediate molecular weight acid, about 0 to 15, e.g. 6 to 12 parts by weight of low molecular weight fatty acid; and sufficient metal base to substantially neutralize said acid mixture.

The lubricating oil used in the compositions of the invention may be either a mineral lubricating oil or a synthetic lubricating oil. Synthetic lubricating oils which may be used include esters of monobasic acids (e.g. C<sub>8</sub> Oxo alcohol ester of C<sub>8</sub> Oxo acid); esters of dibasic acids (e.g. di-2-ethyl hexyl sebacate); esters of glycols (e.g. C<sub>13</sub> Oxo acid diester of tetraethylene glycol); complex esters (e.g. the complex ester formed by reacting one mole of sebacic acid with two moles of tetraethylene glycol and two moles of 2-ethyl-hexanoic acid); esters of phosphoric acid (e.g. the ester formed by contacting three moles of the monomethyl ether of ethylene glycol with one mole of phosphorus oxychloride, etc.); halocarbon oils (e.g. the polymer of chlorotrifluoroethylene containing twelve recurring units of chlorotrifluoroethylene); alkyl silicates (e.g. the methyl polysiloxanes); sulfite esters (e.g. ester formed by reacting one mole of sulfur oxychloride with two moles of the methyl ether of ethylene glycol, etc.); carbonates; mercaptals; formals; etc.

Various other additives may also be added to the lubricating composition (e.g. 0.1 to 10.0 weight percent based on the total weight of the composition), for example, detergents such as calcium petroleum sulfonate; oxidation inhibitors such as phenyl alpha naphthylamine; viscosity index improvers such as polyisobutylene; corrosion inhibitors; such as sorbitan monooleate; pour depressants; dyes; other grease thickeners and the like.

In general, the compositions of the invention will be prepared by coneutralization of the carboxylic acids and the phosphonic or phosphinic acid in situ in a lubricating oil menstruum, by the addition of a metal base, followed by heating to a temperature and for a time necessary to form the complex. Generally the mixture will be heated to about 400° to 700° F., e.g. about 430° to 60° F. The temperature may then immediately be allowed to drop, but preferably is maintained for 1/2 to 4 hours, e.g. 1 to 3 hours in order to ensure the completion of the complex formation. The mixture may then be cooled to about 18 to 200° F., where conventional additives, if any, may be added. The mixture may then be homogenized such as by passing through a Gaulin homogenizer or a Charlotte mill, followed by subsequent cooling to room temperature. The lubricating compositions may also be formed by heating the preformed salts together in the lubricating oil to complexing temperatures.

The invention will be further understood by the following examples which include the preferred embodiments of the invention.

#### EXAMPLE I

A grease was prepared by adding 4 weight percent of 1-hydroxy-1-methylethyl phosphonic acid and 20 weight percent of Hydrofol Acids 51 (hydrogenated fish oil acids

corresponding in degree of saturation and acid number to commercial stearic acid) to 72.7 weight percent of mineral lubricating oil (naphthenic oil having a viscosity of 55 S.U.S. at 210° F.). This mixture was heated in a fire-heated kettle to about 150° F. At this point, a 40% aqueous solution of sodium hydroxide was added in an amount equivalent to 5.3 weight percent of sodium hydroxide and the mixture was further heated to 460° F. Heating was then discontinued and the grease cooled, while agitating, at the rate of 5° F. per minute to 200° F. One weight percent of phenyl alpha naphthylamine was next added and the grease was passed through a Gaulin homogenizer operating at 6000 p.s.i., then cooled to room temperature.

#### EXAMPLE II

Example II was prepared in the same manner as Example I, except that the proportions of the components were changed as shown in Table I.

#### EXAMPLES III TO V

These examples were prepared by charging hydrated lime, mineral oil, Hydrofol Acid 51 and the phosphonic acid to a fire-heated kettle, where the components were thoroughly mixed without external heating. Acetic acid was added to the mixture, which was further stirred for 1/2 hour. The mixture was then heated to 460° F. at a rate of about 3° F./minute. Heating was then discontinued and the grease was allowed to cool to 250° F., at which point phenyl alpha naphthylamine was dispersed in the grease. The grease was further cooled to 150° F., then passed through a Gaulin homogenizer operating at 6000 p.s.i., and finally cooled to room temperature.

#### EXAMPLES VI TO VIII

More fluid lubricants were prepared by further mixing the greases of Examples III to V respectively with an additional portion of mineral lubricating oil.

#### EXAMPLE IX

A grease was prepared by charging mineral oil and lime to a fire-heated kettle and intimately mixing them. To this mixture was added a blend of 12 weight percent glacial acetic acid, 3 weight percent 1-hydroxy-1-methylethyl phosphonic acid and 3 weight percent Wecoline AAC Acid (16 weight percent lauric acid, 28 weight percent caprylic acid and 56 weight percent capric acid). After the acid blend was stirred in, heating was initiated and the mixture was heated to 460° F. Heating was then discontinued and the grease cooled to 200° F., at which point the phenyl alpha naphthylamine was added. The product was then cooled to 150° F. and passed through a Gaulin homogenizer operating at 6,000 p.s.i. The product was cooled to room temperature.

The compositions and properties of Examples I to IX are summarized in Tables I and I-A, which follow.

Table I

| Components (weight percent)                                                            | Example |       |       |        |       |       |        |       |        |
|----------------------------------------------------------------------------------------|---------|-------|-------|--------|-------|-------|--------|-------|--------|
|                                                                                        | I       | II    | III   | IV     | V     | VI    | VII    | VIII  | IX     |
| 1-hydroxy-1-methylethyl phosphonic acid...percent                                      | 4.0     | 2.0   | 1.0   | 2.0    | 3.0   | 0.5   | 1.0    | 1.5   | 3.0    |
| Hydrofol acids 51.....do.....                                                          | 20.0    | 10.0  | 5.0   | 4.0    | 3.0   | 2.5   | 2.0    | 1.5   | 3.0    |
| Wecoline AAC acid <sup>1</sup> .....do.....                                            |         |       | 12.0  | 12.0   | 12.0  | 6.0   | 6.0    | 6.0   | 12.0   |
| Glacial acetic acid.....do.....                                                        | 5.3     | 2.7   | 9.6   | 10.0   | 10.5  | 4.8   | 5.0    | 5.3   | 10.5   |
| Sodium hydroxide.....do.....                                                           |         |       | 1.0   | 1.0    | 1.0   | 0.5   | 0.5    | 0.5   | 1.0    |
| Hydrated lime.....do.....                                                              |         |       |       |        |       |       |        |       |        |
| Phenyl $\alpha$ naphthylamine.....do.....                                              | 1.0     | 1.0   | 1.0   | 1.0    | 1.0   | 0.5   | 0.5    | 0.5   | 1.0    |
| Mineral lubricating oil:                                                               |         |       |       |        |       |       |        |       |        |
| 55 S.U.S. vis. at 210° F.....do.....                                                   | 69.7    | 84.3  | 71.4  | 71.0   | 70.5  | 35.7  | 35.5   | 35.2  | 70.5   |
| 80 S.U.S. vis. at 210° F.....do.....                                                   |         |       |       |        |       | 50.0  | 50.0   | 50.0  |        |
| Mole ratio of high or intermediate molecular weight fatty acid to phosphonic acid..... | 2.5/1   | 2.5/1 | 2.5/1 | 1/1    | 5/1   | 2.5/1 | 1/1    | 0.5/1 | 1.13/1 |
| Mole ratio of acetic acid to phosphonic acid.....                                      |         |       | 29/1  | 14.5/1 | 9.5/1 | 29/1  | 14.5/1 | 9.6/1 | 9.5/1  |

<sup>1</sup> 16% lauric acid; 28% caprylic acid; 56% capric acid.

Table I-A

| Properties                                                                | Example                                  |        |        |        |        |      |      |      |       |
|---------------------------------------------------------------------------|------------------------------------------|--------|--------|--------|--------|------|------|------|-------|
|                                                                           | I                                        | II     | III    | IV     | V      | VI   | VII  | VIII | IX    |
| Appearance                                                                | Excellent, smooth, homogeneous lubricant |        |        |        |        |      |      |      |       |
| Dropping point, °F.                                                       | 500+                                     | 500+   | 500+   | 500+   | 500+   | 500  | 500  | 500  |       |
| Penetration 77° F., mm./10—                                               |                                          |        |        |        |        |      |      |      |       |
| Unworked                                                                  | 192                                      | 275    | 195    | 300    | 350    | 360  | 380  | (1)  |       |
| Worked 60 strokes                                                         | 202                                      | 285    | 200    | 310    | (1)    | (1)  | (1)  |      |       |
| Worked 100,000 strokes (fine hole worker plate)                           | 215                                      | 290    | 195    | 235    |        |      |      |      |       |
| Thixotropy and effect of temperature                                      | Not thixotropic                          |        |        |        |        |      |      |      |       |
| Penetrations at 300° F.                                                   | Good thixotropy <sup>2</sup>             |        |        |        |        |      |      |      |       |
| Crust formation                                                           | None                                     | None   | Slight | None   | None   | 320  | 340  | 375  | None  |
| Water solubility (boiling water):                                         | Up to 150° F.                            |        |        |        |        |      |      |      |       |
| Above 150° F.                                                             | Insol.                                   | Insol. | None   | None   | None   |      |      |      |       |
| Viscosities S.U.S. at                                                     | 100° F.                                  |        |        |        |        |      |      |      |       |
| 100° F.                                                                   |                                          |        |        |        |        |      |      |      | 2,100 |
| 210° F.                                                                   |                                          |        |        |        |        |      |      |      | 200   |
| Transition point on heating                                               |                                          |        |        |        |        |      |      |      |       |
| Stability of dispersion                                                   | Excellent <sup>7</sup>                   |        |        |        |        |      |      |      |       |
| Extreme pressure properties: Almen Tests—                                 |                                          |        |        |        |        |      |      |      |       |
| Wgts. carried (gradual load)                                              |                                          |        | 15     | 15     | 15     | 13   | 15   | 15   | 15    |
| Wgts. carried (shock loading)                                             |                                          |        | 15     | 15     | 15     |      | 15   | 15   | (8)   |
| Pin Condition                                                             |                                          |        |        |        |        |      |      |      |       |
| 4 ball wear test scar spot dia. mm. (1,800 R.P.M.-10 kg.—1 hr. at 75° C.) | 0.45                                     | 0.40   | 0.22   | 0.20   | 0.22   | 0.28 | 0.20 | 0.20 | 0.24  |
| Timken machine test, 45 lbs. load                                         | Pass                                     |        |        |        |        |      |      |      |       |
| Norma Hoffmann oxidation hours to 5 p.s.i. drop                           | 400+                                     | 400+   | 300    | 400    | 385    |      |      |      |       |
| Lubrication life (hours) 250° F.-10,000 r.p.m.                            | 9 2,500                                  |        | 3,200+ | 1,500+ | 3,000+ |      |      |      |       |

<sup>1</sup> Semifluid.<sup>2</sup> Tends to set up harder after working.<sup>3</sup> Sets up solid on removal of shearing stress. Also tends to become harder on increasing temperature.<sup>4</sup> Slowly disintegrates.<sup>5</sup> Disintegrates.<sup>6</sup> Remains fluid up to 400° F.<sup>7</sup> No tendency to separate after 14 days at 210° F.<sup>8</sup> Excellent, polished.<sup>9</sup> Still running.

As seen from the above table, excellent high temperature lubricants, having high dropping points and excellent extreme pressure and anti-wear properties may be formed from complexes of the salts of the phosphonic acid in various combinations with salts of fatty acid.

Examples I and II illustrate the use of the phosphonic acid and high molecular weight fatty acids. These complexes had 4-ball wear scar diameters of 0.45 to 0.04 mm. respectively, which is very good as prior commercial greases thickened with sodium complexes of comparable amounts of high molecular weight fatty acid and acetic acid have wear scar diameters of about 0.65 mm. Also, the sodium greases of Examples I and II were water-insoluble up to 150° F., which was surprising in view of the fact that sodium greases are invariably water-soluble at much lower temperatures.

Examples III to V illustrate calcium complex greases containing the phosphonic acid, high molecular weight fatty acid and acetic acid. These greases illustrate particularly preferred compositions of the invention since they had a high degree of thixotropy, i.e., they quickly revert to their solid form upon removal of shearing stresses, and also had very good extreme pressure and anti-wear properties. Furthermore, the greases of Examples III to V had either a very slight or no tendency at all to form a crust, while prior comparable greases containing complex salts of Hydrofolic Acids 51 and acetic acid (e.g. in a 1/1 molar ratio) excessively harden on exposure to air to form undesirable crusts. Examples III to V also illustrate the fact that by holding the proportion of acetic acid constant, and increasing the ratio of the phosphonic acid to the high molecular weight fatty acid, that products of increasing fluidity are obtained. This concept is of particular importance as it permits the formation of more fluid products which still have a high soap and

correspondingly, a high metal content which imparts high extreme pressure properties to the lubricant. Generally, in the past, it was common practice to increase the extreme pressure properties of a lubricant by increasing the soap content, however, this was rather a limited procedure since the increased soap content would unduly harden the grease. However, a method has now been found for obtaining good wear and extreme pressure properties and yet still be able to control the plasticity or fluidity of the grease.

Examples VI to VIII illustrate the use of decreasing amounts of the complex to form more fluid lubricants having high extreme pressure properties and low wear characteristics. Even these diluted materials illustrated some degree of thixotropy. The lubricant of Example VIII, upon further dilution with an equal amount of mineral oil (80 S.U.S. at 210° F.) still carried 8 Almen weights upon gradual loading and in a 4-ball wear test gave a .20 mm. dia. scar. These fluid and semi-fluid lubricants are particularly valuable for certain applications, as in upper cylinder lubrication of diesel engines where extreme pressure and anti-wear properties are necessary to prevent cylinder liner and ring wear. In view of the current tendency to burn the more economical high sulfur-containing residual fuel oils in diesel engines, these lubricants are particularly good as they have a high degree of neutralization potential present, i.e. the calcium acetate portion of the complex will neutralize H<sub>2</sub>SO<sub>4</sub> formed by the burning of the sulfur in the fuel. The soap or grease therefore present on the surface of the liner and rings also protects the metal from acid corrosion.

Example IX illustrates a fluid lubricant prepared from the phosphonic acid, acetic acid, and a mixture of intermediate molecular weight fatty acids. Example IX is similar to Example V, the only difference being the use

of the intermediate molecular weight fatty acid instead of high molecular weight fatty acid. These examples illustrate the fact that more fluid products may also be obtained by using lower molecular weight fatty acids.

It had been known to form complex thickeners comprising salts of a high molecular weight fatty acid and salts of acrylic acid by heating whole fat such as tallow, hog fat, lard oil, fish oil, or vegetable oils as rapeseed oil, mustard seed oil, etc., to high temperatures in the presence of a large excess of alkali, such as sodium or potassium alkali. The fat becomes saponified at about 350° F., then upon further heating to about 500° F., a portion of the fat breaks down to form glycerine which is dehydrated to acrolein which, in turn, is converted into salts of acrylic acid. However, the large excess of alkali necessary for such reactions tends to make the grease more abrasive and therefore undesirable from a dermatitis standpoint. It has now been found that by neutralizing the excess alkali with the phosphonic acids of the invention such as 1-hydroxy-1-methylethyl phosphonic acid, that the extreme pressure and anti-wear properties of the grease are much improved along with highly improved resistance to oxidation, while the abrasiveness due to the excess alkali is eliminated. This concept of the invention is illustrated by the following examples.

Greases of the above type are readily prepared by dispersing a fat in lubricating oil, adding about 1.5 to 3.0 times the amount of alkali necessary for saponification, heating to a temperature of about 450 to 650° F., e.g. 500 to 550° F., for about 10 to 30 minutes, or until foaming due to hydrogen evolution ceases, cooling to about 250 to 300° F., then adding sufficient 1-hydroxy alkyl phosphonic acid to neutralize any excess alkali, then maintaining a temperature of about 200 to 400° F., e.g. 250 to 300° F. for about 20 to 45 minutes in order to ensure the complete reaction of the phosphonic acid with the excess alkali, followed by cooling to room temperature.

#### EXAMPLE X-A

A grease was prepared by charging mustard seed oil, mineral oil and sodium petroleum sulfonate (ave. mol. wt.—480) to a kettle and then warming to 150° F., while mixing. A 40 percent aqueous solution of sodium hydroxide was added to the kettle and the contents further heated. Dehydration and foaming then occurred, which ceased at temperatures of about 350° F. On continued heating to 450° F., foaming again began due to hydrogen evolution. Heating was continued to 520° F. and the temperature maintained there for about 30 minutes, until foaming ceased. Heating was discontinued and the temperature was allowed to drop to 300° F., at which point the hydroxy phosphonic acid was added. The mixture was maintained at 300° F. for about 30 minutes. Then phenyl alpha naphthylamine was added and the grease cooled to 150° F. where it was passed through a Gaulin homogenizer operating at 6,000 p.s.i. The grease was then cooled to room temperature.

#### EXAMPLE X-B

A grease similar to that of Example X-A was prepared, except that the excess alkalinity was not neutralized with phosphonic acid.

#### EXAMPLE XI

The grease of Example X-A was further diluted with 25 weight percent of additional mineral oil.

The compositions of the above greases and their physical properties are shown in Table II.

8  
Table II

|    | Components (parts by weight)                                                   | Example |       |       |
|----|--------------------------------------------------------------------------------|---------|-------|-------|
|    |                                                                                | X-A     | X-B   | XI    |
| 5  | Mustard seed oil.....                                                          | 22.00   | 22.00 | 16.50 |
|    | Sodium hydroxide.....                                                          | 4.95    | 4.75  | 3.71  |
|    | Sodium sulfonate.....                                                          | 1.00    | 1.00  | .75   |
| 10 | Mineral lubricating oil (55 S.U.S. at 210° F.)                                 | 70.55   | 77.25 | 77.17 |
|    | 1-hydroxy-1-methylethyl phosphonic acid.....                                   | 1.50    | —     | 1.12  |
|    | Phenyl alpha naphthylamine.....                                                | 1.00    | 1.00  | .75   |
|    | Properties                                                                     |         |       |       |
| 15 | Appearance.....                                                                | (1)     | (1)   | (1)   |
|    | Dropping point, ° F.....                                                       | 500+    | 500+  | 480   |
|    | Penetration 77° F. mm./10:                                                     |         |       |       |
|    | Unworked.....                                                                  | 175     | —     | 265   |
|    | Worked 60 strokes.....                                                         | 180     | 275   | 275   |
|    | Worked 100,000 strokes.....                                                    | 195     | 340   | 325   |
| 20 | Lubrication test* (204 bearing—10,000 r.p.m.), time and temperature rise.....  | (2)     | (2)   | (2)   |
|    | 4-ball wear test scar dia., mm. (1,800 r.p.m.—10 kg. Id.—1 hr. at 75° C.)..... | 0.40    | 0.65  | 0.35  |
|    | Color stability, 3 weeks at 250° F.....                                        | (4)     | (3)   | (4)   |
|    | Normal Hoffman oxidation, hours to 5 p.s.i. drop.....                          | 305     | 225   | 350   |

<sup>1</sup> Excellent, smooth grease.

<sup>2</sup> Anti-Friction Bearing Manufacturers Association—National Lubricating Grease Institute Cooperative Test for Lubrication Life.

<sup>3</sup> 10 min., 50° F. rise.

<sup>4</sup> Excellent, no crust formation or darkening of grease.

<sup>5</sup> Poor—dark. Slight crust formation.

As seen from the above data, the greases prepared from the phosphonic acid had low wear scar diameters, better color stability and were more resistant to oxidation than a similar grease which did not contain the phosphonic acid.

While the preceding examples utilized a purified 1-hydroxy-1-methylethyl phosphonic acid, it was also found that a crude phosphonic acid product resulting from the commercial preparation of the acid is suitable and can be more easily and less expensively manufactured. Thus in the commercial preparation of the acid, equal molar quantities of a ketone, e.g. acetone, and phosphorous trichloride were reacted together. Acetic acid in excess of 2 moles was then added and the acetyl chloride and HCl which formed were removed by vacuum distillation. The resulting phosphonic acid material was then hydrolyzed and recrystallized from the excess acetic acid. It has now been found that after distillation to remove the HCl and acetyl chloride, the crude dispersion or solution of the phosphonic acid in acetic acid may be employed directly in preparing the grease. This concept is illustrated by the following example.

#### EXAMPLE XII

A 5-liter 4-necked flask equipped with a stirrer, condenser, thermometer and dropping funnel was charged with 209 g. acetone (3.6 m.) and 412 g.  $\text{PCl}_3$  (3.0 m.). This mixture was stirred for 5 minutes, then allowed to stand overnight (16 hours) at room temperature. It was then cooled to 55° F. and maintained at 55° to 65° F. while 720 g. of glacial acetic acid was added over a 45 minute period. Stirring was continued at this temperature for another 2 hours, after which the total product was transferred to a distillation flask and stripped in a short path still. The first part of the stripping was at atmospheric pressure until most of the HCl gas and acetyl chloride had been removed. Reduced pressure was then applied and the product stripped to a pot temperature of 93° C. with the vapor temperature at 65° C. under 2.5 mm. Hg. This left a residue of 467 g. having a neut. number of 819.3 mg. KOH/gm. crude material.

The residue obtained above and consisting of about 70 wt. percent crude phosphonic acid and 30 wt. percent

acetic acid was then used to prepare a grease having the following composition:

|                                                                 | Percent |
|-----------------------------------------------------------------|---------|
| Glacial acetic acid                                             | 11.4    |
| Hydrofol acids 51                                               | 6.0     |
| 70% crude phosphonic acid in acetic acid                        | 1.6     |
| Hydrated lime                                                   | 9.8     |
| Phenyl $\alpha$ -naphthylamine                                  | 1.0     |
| Mineral lubricating oil having a viscosity of 55 SUS at 210° F. | 70.2    |
|                                                                 | 10      |

This grease was prepared by charging the lime, mineral oil, Hydrofol Acids 51, and the crude phosphonic acid to a fire heated kettle and intimately mixing. The glacial acetic acid was then added and the mixture was heated to 460° F. Then, the grease was cooled to 200° F., the phenyl  $\alpha$ -naphthylamine added and further cooled to 150° F. where the solid grease base was Gaulin homogenized at 6,000 p.s.i., then cooled to room temperature.

The homogenized base material prepared above was then further blended with varying amounts of mineral lubricating oils as shown in the following table:

Table III

| Components (weight percent)                         | Example XII       |                   |                   |                            |
|-----------------------------------------------------|-------------------|-------------------|-------------------|----------------------------|
|                                                     | A                 | B                 | C                 | D                          |
| Base composition <sup>1</sup>                       | 50.               | 60.               | 70.               | 60.                        |
| Mineral lubricating oil (80 SUS at 210° F.)         | 50.               | 40.               | 30.               |                            |
| Mineral oil bright stock (about 191 SUS at 210° F.) |                   |                   |                   | 40.                        |
| Properties                                          |                   |                   |                   |                            |
| Appearance                                          | Excellent         | Excellent         | Excellent         | Excellent                  |
| Dropping point F.                                   | 500+              | 500+              | 500+              | 500+                       |
| Penetration 77° F. mm./10:                          |                   |                   |                   |                            |
| Unworked                                            | 360.              | 320.              | 300.              | 320.                       |
| Worked 60 strokes                                   | Semi-fluid        | Semi-fluid        | Semi-fluid        | 380 to fluid. <sup>2</sup> |
| Time to recover to original consistency             | 10 min.           | 3 min.            | 15 secs.          | Instantaneous              |
| 4-ball wear test scar spot dia. mm.                 | 0.25.             | 0.28.             | 0.24.             |                            |
| Stability                                           | Good <sup>3</sup> | Good <sup>3</sup> | Good <sup>3</sup> |                            |

<sup>1</sup> Base composition prepared from 11.4% glacial acetic acid, 6% hydrofol acids 51, 1.6 weight percent of phosphonic acid in acetic acid solution, 9.8% hydrated lime, 1.0% phenyl  $\alpha$ -naphthylamine, and 70.2% mineral oil.

<sup>2</sup> Fluid while mixing or exerting shearing stress.

<sup>3</sup> No tendency to solidify or crust formation after storage for 30 days.

As seen from the above compositions, greases having varying degrees of thixotropy may be prepared from the crude phosphonic acid. For comparison, a composition similar to that of Example XII-A was prepared using the purified acetone hydroxy phosphonic acid instead of the corresponding crude phosphonic acid. However, there were no significant differences between the properties of the two compositions.

To illustrate the use of a phosphinic acid in preparing the grease compositions of the invention, the following example was carried out:

## EXAMPLE XIII

A. A grease was prepared having the following composition:

|                                           | Percent |
|-------------------------------------------|---------|
| Glacial acetic acid                       | 12.0    |
| Hydrofol acids 51                         | 5.0     |
| 1-hydroxy-1-methyl propyl phosphinic acid | 1.0     |
| Hydrated lime                             | 9.6     |
| Phenyl $\alpha$ -naphthylamine            | 1.0     |
| Diol 55                                   | 71.4    |

The grease was made as follows: Lime, Hydrofol Acids 51, and mineral oil were added to a fire heated kettle and mixed thoroughly to an intimate smooth slurry. A blend of the phosphinic acid and acetic acid was added, followed by stirring for  $\frac{1}{2}$  hour. After this period, heating was begun and the temperature was raised to 460° F. The heat was turned off, the mixture cooled to 200° F., while stirring and phenyl  $\alpha$ -naphthylamine was added, followed by continued mixing and cooling to 150° F.,

where the grease was Gaulin homogenized at 6000 p.s.i. before being cooled to room temperature. The resulting grease had the following properties:

Appearance—excellent, smooth uniform grease

5 Dropping point—500° F.+

Penetration, 77° F., mm./10:

Unworked—240

Worked, 60 strokes—under shearing stress the grease becomes semi-fluid. Upon removal of stress the grease hardened immediately.

B. 80 wt. percent of the grease prepared above was diluted with 20 wt. percent of additional mineral lubricating oil (80 SUS at 210° F.), then Gaulin homogenized at 5000 p.s.i. A smooth solid grease resulted having an A.S.T.M. unworked penetration of 310 mm./10 at 77° F.; a high degree of thixotropy; good storage stability; and which carried 15 Almen weights and gave a wear scar dia. of 0.25 in the 4-ball wear test.

20 What is claimed is:

1. A lubricant composition comprising a major proportion of lubricating oil and an extreme-pressure imparting amount of a mixed-salt complex material com-

45 prising metal salts of fatty acids selected from the group consisting of intermediate and high molecular weight fatty acids and mixtures thereof, and metal salts of a phosphorus containing acid containing 1 to 5 carbon atoms selected from the group consisting of 1-hydroxy alkyl phosphonic acid and 1-hydroxy alkyl phosphinic acids, wherein the molar ratio of said fatty acids to said phosphorus-containing acid is about 0.1 to 10.0 moles of fatty acid per mole of said phosphorus-containing acid and wherein said metal is selected from the group consisting of alkali metals and alkaline earth metals.

50 2. A lubricant composition according to claim 1, which contains about 5 to 30 weight percent, based on the total composition, of said complex material.

3. A lubricant composition according to claim 1, where- 55 in said fatty acid comprises a mixture of C<sub>7</sub> to C<sub>12</sub> fatty acid and C<sub>16</sub> to C<sub>30</sub> fatty acid.

4. A lubricant composition according to claim 1, where- 60 in said phosphorus-containing acid is a phosphinic acid.

5. A lubricant composition according to claim 1, where- 65 in said phosphorus-containing acid is a phosphonic acid.

6. A lubricant composition according to claim 1, where- 70 in said mixed-salt complex includes salts of C<sub>1</sub> to C<sub>6</sub> fatty acid in a molar ratio of said C<sub>1</sub> to C<sub>6</sub> fatty acid to said phosphorus-containing acid of about 5:1 to 30:1.

7. A lubricant composition according to claim 1, where- 75 in said oil is a mineral oil.

8. A lubricating composition comprising a major proportion of lubricating oil and about 5 to 30 weight percent, based on the total composition, of a thickener com- 75 prising, in a molar ratio, metal salt of about 0.5 to 30.0

## 11

moles of  $C_1$  to  $C_6$  fatty acid, metal salt of about .1 to 10 moles of fatty acid selected from the group consisting of  $C_7$  to  $C_{12}$  fatty acid and  $C_{16}$  to  $C_{30}$  fatty acid, and mixtures thereof, and metal salt of one mole of a phosphorus-containing acid selected from the group consisting of 1-hydroxy alkyl phosphonic and 1-hydroxy alkyl phosphinic acid containing 1 to 5 carbon atoms, and wherein said metal is selected from the group consisting of alkali and alkaline earth metals.

9. A lubricating composition comprising a major proportion of lubricating oil and 5 to 30 weight percent of a thickener which comprises metal salts of: 2 to 5 parts by weight of a  $C_1$  to  $C_5$  of an organic phosphorus-containing acid selected from the group consisting of 1-hydroxy alkyl phosphonic acid and 1-hydroxy alkyl phosphinic acid, 1 to 20 parts by weight of fatty acid selected from the group consisting of  $C_7$  to  $C_{12}$  fatty acid and  $C_{16}$  to  $C_{30}$  fatty acid and mixtures thereof, and 0 to 15 parts by weight of  $C_1$  to  $C_6$  fatty acid, wherein said metal is selected from the group consisting of alkali metals and alkaline earth metals.

10. A process for the preparation of lubricants which comprises conneutralizing with a metal base a dispersion of fatty acid selected from the group consisting of  $C_7$  to  $C_{12}$  fatty acids,  $C_{16}$  to  $C_{30}$  fatty acids and mixtures thereof, and a phosphorus-containing acid selected from the group consisting of 1-hydroxy alkyl phosphonic and phosphinic acids in lubricating oil, then heating to a temperature of about 400 to 700° F. and then cooling, said metal base being selected from the group consisting of alkaline earth metal bases.

11. A process for the preparation of a lubricant which comprises reacting a dispersion of whole fat in lubricating oil with about 1.5-3.0 times the amount of alkali

5

10

15

20

25

30

## 12

needed for complete saponification of said fat at temperatures of about 450 to 650° F. until foaming substantially ceases, cooling to about 200 to 400° F., then neutralizing said excess alkali with a phosphorus-containing acid selected from the group consisting of 1-hydroxy-alkyl phosphonic and phosphinic acids before final cooling to form said grease.

12. A lubricant composition comprising lubricating oil and about 5 to 30 wt. percent, based on the total composition, of a mixed-salt material comprising metal salts of a fatty acid selected from the group consisting of  $C_7$  to  $C_{12}$  and  $C_{16}$  to  $C_{30}$  fatty acids and metal salts of a crude  $C_1$  to  $C_5$  1-hydroxy alkyl phosphonic acid material comprising a solution of said phosphonic acid in acetic acid obtained by reacting a ketone and  $PCl_3$ , adding acetic acid in excess and distilling to remove  $HCl$  and acetyl chloride to leave said crude phosphonic acid as a residue, wherein the molar ratio of said fatty acids to said phosphonic acid is about 0.1 to 10.0 moles of fatty acid per mole of said phosphonic acid and wherein said metal is selected from the group consisting of alkali metals and alkaline earth metals.

## References Cited in the file of this patent

## UNITED STATES PATENTS

|           |               |               |
|-----------|---------------|---------------|
| 2,513,680 | Schott et al. | July 4, 1950  |
| 2,628,949 | Butcosk       | Feb. 17, 1953 |
| 2,758,971 | Mikeska       | Aug. 14, 1956 |
| 2,837,481 | Hotten et al. | June 3, 1958  |
| 2,846,392 | Morway et al. | Aug. 5, 1958  |

## FOREIGN PATENTS

|         |               |               |
|---------|---------------|---------------|
| 549,296 | Great Britain | Nov. 16, 1942 |
|---------|---------------|---------------|